

## UNITED STATES PATENT OFFICE.

WILLIAM P. BENTLEY, OF DALLAS, TEXAS.

## TREATMENT OF ROCK ASPHALT.

No Drawing.

Application filed February 17, 1928. Serial No. 255,202.

This application is a continuation in part of my co-pending application, Serial No. 152,723.

The present invention has for its principal objects the improvement in methods for the commercial utilization of naturally occurring rock asphalt, and the improvement thereby of the quality of the product for which the material is to be adapted. The principal use of the material here contemplated is for that of paving streets, roadways, highways, foot-paths, mastics for floorings, roofings, and the like, but in its broader aspects might be utilized for any purpose for which asphaltic materials have been used.

Rock asphalts are found in a great variety of forms and in various localities, and are both siliceous and calcareous in body impregnated with bituminous material ranging from very hard to very soft. By far the greater percentage of these rock asphalts is of such composition that they cannot be used per se for pavements, but require pre-treatment to some extent. This treatment may comprise crushing the rock asphalt, the liquefaction of the self-contained bitumen either by means of heat or by a solvent and the subsequent or simultaneous addition of a bituminous flux for the purpose of softening or hardening the bitumen and at the same time increasing the bitumen content to that desired in the final pavement.

Heretofore the methods used for regulating the crushing operation and for computing the proper amount and kind of bituminous flux for the production of the greatest stability or strength in the final pavement has been entirely haphazard and mere guess work. As an illustration of the present state of the art, in a bulletin issued September 1, 1926, by the A. & M. College of Texas, J. T. L. McNew, professor of highway engineering, after an exhaustive discussion of Texas rock asphalts, concludes that "The proper fluxing of the bitumen in Texas limestone rock asphalt that is lean in natural asphalt content is a problem which cannot be solved without further investigation." It is precisely such an extensive investigation carried on by me over a

period of years which has led to the concept which is the embodiment of this invention.

The specific feature of this invention is primarily that of regulating the voidage in the crushed rock asphalt aggregate, either by the crushing operation itself, or by the addition of certain desirable size of bitumen-free or bitumen-impregnated particles, or by both. Concurrently with this, by knowing or pre-determining voidage, the selection of the suitable flux for imparting the desired hardness or softness to the naturally contained bitumen becomes a matter of scientific control, and is always productive of improved quality to the final product. This combination of voidage regulation, flux consistency, and quality control, has never been known before, nor has it ever been possible before to pre-determine the stability of the final composition. With a given kind of rock asphalt which may have been in use for a long period of years, experience may have led to very successful results for varieties of conditions. Even current practice which has given practical results, can be greatly improved by application of my method and mixtures can then be controlled as to characteristics heretofore mentioned. But when attempting to open new deposits or to work with different kinds of rock asphalts, nothing in past experience would be available, hence controlled stability would be a matter of assumption or mere guess work. This invention also opens up vast fields of rock asphalt which have been considered as inadequate and inferior on account of not lending itself to successful operation when the same kind of flux as is ordinarily used, is employed; likewise, rock asphalts carrying bitumen of different degrees of consistency were not deemed satisfactory for the usual given method of treatment. In order to illustrate one method of using this invention, a description of design in a mixture for paving purposes may be given; this refers to a particular kind of rock asphalt found in Texas, but in no manner limits this invention to such particular kind of rock asphalt or particular kind of usage.

The rock asphalt is crushed in any ordinary type of mill or roll, and with its self-

contained bitumen constituting the aggregate, its voidage is determined by compaction to refusal in any of the usual instruments for such a determination. Then various proportions of previously separated particles, for instance, 200 mesh sizes, or 80 mesh, or 40 mesh, or 10 mesh, or such, may be added in progressive increments until the minimum practicable combination of voids 5 for workability is produced. From this voidage and the specific gravity of the rock asphalt, the amount of bitumen necessary to be added to fill said voids can be readily computed. With this valuable information 10 the kind of bitumen to be added to keep the resulting consistency of the final product within specified limits can be determined by simple fluxing tests. Then, by determining the stability values of compressed mixtures 15 either by shear tests, or other such method, a pre-determined service record will be available. By knowing the traffic, climatic conditions, etc., to be encountered, any of the above factors can be regulated or adjusted 20 to meet the proposed need. I have discovered that the highest practicable shear values are obtained by so regulating the bitumen that the voids in the final composition, after compression, are just filled. 25 Which, stated in another way, means that the amount of bitumen in the final mixture is regulated by adding, if necessary, a flux in such an amount that, when taken in conjunction with the self-contained bitumen in 30 the rock, fills the voids without substantial excess or deficiency.

The most common failure which might be found inherent in an asphaltic pavement is that of distortion, and since the distorting 40 forces of traffic are mainly shear, it can be seen that resistance to shear is a direct measurement of the resistance of a pavement to distortion.

From the above it is believed that those 45 skilled in the art will be taught how to obtain the highest practicable shear values. The engineer knows that the rock asphalt contains naturally a certain amount of bitumen to which a flux must be added in 50 order that the sum may fill the voids. The part added must be less than the sum so that it naturally follows that the flux itself is insufficient to fill the voids. Mathematically he computes the above named quantities 55 as follows:

Let  $F$ —percent flux required,  
and  $V$ —percent voids found in crushed rock asphalt.

$P$ —percent bitumen naturally contained 60 in the rock asphalt.

$T$ —percent total bitumen in mixture computed to fill voids.

$S$ —Specific gravity of mineral in the rock asphalt.

$s$ —Specific gravity of the bitumen in the mixture.

Then in the mixture which being designed according to this method

$V_s$ —relative weight of bitumen in the mixture.

$(1-V_s)$   $S$ —relative weight of mineral in the mixture.

$V_s + (1-V_s)S$ —relative weight of mixture.

$$T = \frac{V_s}{V_s + (1-V_s)S}$$

Therefore  $F$  equals  $T$  minus  $P$ .

All the examples lettered from A to G given hereinafter are figured as outlined above. Take Example "A". It is stated that:

(V) Percent voids in rock asphalt as used=23.2.

(P) Percent bitumen in rock asphalt=8 to 9.

T Percent computed bitumen content required=10.35.

"(Percentage total bitumen required to fill voids in aggregate)." 90

The mixture actually contained 10.3% bitumen.

What amount of flux was added? Obviously, it was 10.3% minus the percent bitumen already contained in the rock. In other words, 1.3% to 2.3% would be required for rock asphalt containing 8 to 9 percent bitumen. 95

Not only does this above outlined procedure enhance the quality of known rock asphalts, but it also opens up for use other vast deposits which have been ignored for supposed lack of sufficient bitumen, or seemingly improper degree of crushing resistance, or too hard or too soft self-contained bitumen, or a combination of these qualities, which by my treatment are rendered highly satisfactory. 100

The following tabulation will assist in an understanding of the present invention: 105

#### EXAMPLE A.

Regular run Uvalde rock asphalt containing 8 to 9% bitumen.

Percentage voids in rock asphalt as used 23.2 115

Sieve analysis of rock asphalt percentage passing 200 mesh 11.0

90 mesh 10.0

40 mesh 20.0 120

10 mesh 41.0

Retained on 10 mesh 18.0

(Refers to voids and grading of crushed rock asphalt with its self-contained bitumen present.) 125

Computed bitumen content required % 10.35

(Percentage total bitumen required to fill voids in aggregate.)

Shear strength at 140° F. in pounds per square inch \_\_\_\_\_ 63.3

5 Mixture analysis (after shearing sample).

Bitumen % \_\_\_\_\_ 10.3  
Per cent passing 200 mesh \_\_\_\_\_ 20.3  
80 mesh \_\_\_\_\_ 14.5  
10 40 mesh \_\_\_\_\_ 19.6  
10 mesh \_\_\_\_\_ 26.8  
4 mesh \_\_\_\_\_ 8.5  
2 mesh \_\_\_\_\_ 0

15 Approximate penetration at 77° of bitumen extracted from mixture \_\_\_\_\_ 60

The mixture actually contained 10.3% bitumen. The flux added was 10.3% minus the percent of bitumen already contained 20 in the rock. In other words 1.3% to 2.3% would be required for rock asphalts containing 8 or 9% bitumen.

#### EXAMPLE B.

25 Regular run Uvalde rock asphalt containing 8 to 9% bitumen with 200 mesh portion increased 10%—no flux used.

Percentage voids in rock asphalt \_\_\_\_\_ 18.3

30 Sieve analysis of rock asphalt percentage passing—  
200 mesh \_\_\_\_\_ 14.5  
80 mesh \_\_\_\_\_ 11.1  
40 mesh \_\_\_\_\_ 19.7  
35 10 mesh \_\_\_\_\_ 40.3  
4 mesh \_\_\_\_\_ 11.1  
2 mesh \_\_\_\_\_ 3.3

40 (Refers to voids and grading of crushed rock asphalt with its self-contained bitumen present).

Computed bitumen content required % \_\_\_\_\_ 7.9

(Percentage total bitumen required to fill voids in aggregate).

45 Shear strength at 140° F. in pounds per square inch \_\_\_\_\_ 190.

Mixture analysis (after shearing sample).

Bitumen % \_\_\_\_\_ 9.0  
50 Percent passing:  
200 mesh \_\_\_\_\_ 24.0  
80 mesh \_\_\_\_\_ 13.9  
40 mesh \_\_\_\_\_ 19.9  
10 mesh \_\_\_\_\_ 24.0  
55 4 mesh \_\_\_\_\_ 9.2  
2 mesh \_\_\_\_\_ 0

Approximate penetration at 77° F. of bitumen extracted from mixture \_\_\_\_\_ 8

60 This example is included to show that when the voids are reduced to 18.3%, rock asphalt containing 8% bitumen already has its voids filled. It is impossible to flux this rock asphalt to raise the penetration of the

65 bitumen to a higher and more desirable

working penetration without overfilling the voids, unless the bituminous content thereof is lowered by blending with leaner rocks or by adding mineral matter. If the penetration of the self-contained bitumen was already at the desired point, all that would be necessary to use this rock under this method would be to reduce the voids until the self-contained bitumen just filled same. The flux to be added in such a case would be 0%. 75

#### EXAMPLE C.

Regular run Uvalde rock asphalt containing 11% total bitumen.

Percentage of voids, sieve analysis, and 80 computed bitumen content required—identical with Example A.

The mixture analysis, however, showed 11% bitumen with a shear of 27.7 and a penetration in excess of 100. 85

Note from Example C what happens to the shear as compared with Example A when the voids are overfilled by the total bitumen. Here the amount of flux added was too much by 0.7%. This mix was made this way purposely for illustration. 90

#### EXAMPLE D.

Using only the same base with only 10% bitumen had a shear strength of 56.5, a bitumen content in the mixture analysis of 9.9 and a penetration of 30. 95

Note from this example what happens to the shear when the voids are underfilled by total bitumen. Here the flux added was too little. 100

#### EXAMPLE E.

Special lean Uvalde rock asphalt of 5.5 to 6% bitumen with flux added in an amount sufficient to produce in the final mixture a total bitumen content from .5% to 1.0% in excess of that actually required to fill voids. 105

Percentage voids in rock asphalt \_\_\_\_\_ 18.6  
Sieve analysis of rock asphalt % passing:  
200 mesh \_\_\_\_\_ 13.7  
80 mesh \_\_\_\_\_ 12.9  
40 mesh \_\_\_\_\_ 17.9  
10 mesh \_\_\_\_\_ 39.0  
4 mesh \_\_\_\_\_ 14.8  
2 mesh \_\_\_\_\_ 1.7 115

Computed bitumen content required % \_\_\_\_\_ 8.05

Shear strength at 140° F. in pounds per square inch \_\_\_\_\_ 21.7 120

Mixture analysis (after shearing sample).

Bitumen % \_\_\_\_\_ 8.2  
Percentage passing:  
200 mesh \_\_\_\_\_ 20.7 125  
80 mesh \_\_\_\_\_ 13.3  
40 mesh \_\_\_\_\_ 16.3  
10 mesh \_\_\_\_\_ 28.7  
4 mesh \_\_\_\_\_ 10.6  
2 mesh \_\_\_\_\_ 2.2 130

Approximate penetration at 77° F. of bitumen extracted from mixture—100 plus.

Note from Example E that, when the voids (V) are reduced to 18.6% and the total bitumen is one-half to one percent in excess and using the flux generally used on Texas rock asphalt hot mixes, the shear is only 21.7 pounds. Note how the total bitumen required as computed goes down to 8.05% with lowering of voids. The high penetration accounts for the low shear shown by this example and discloses that when low voidage mixtures are used on Texas rock asphalts, the flux now in general use is not of the right type.

#### EXAMPLE F.

Same as Example E with no excess of flux, using 300 penetration flux showed an increase in shear strength to 111.5, and a decrease in penetration to 26.

#### EXAMPLE G.

Special lean Uvalde rock asphalt of 5.5 to 6% bitumen, with 200 mesh increased 10% and bitumen to fill voids (using 300 penetration flux).

|                                                     |       |
|-----------------------------------------------------|-------|
| Percentage voids in rock asphalt                    | 18.0  |
| Sieve analysis (proportions by weight)              |       |
| bitumen                                             | 7.7   |
| Percentage passing 200 mesh                         | 20.1  |
| 80 mesh                                             | 10.8  |
| 40 mesh                                             | 15.0  |
| 10 mesh                                             | 32.8  |
| 4 mesh                                              | 12.4  |
| 2 mesh                                              | 1.2   |
| Computed bitumen content required                   | 7.7   |
| Shear strength at 140° F. in pounds per square inch | 145.0 |

Mixture analysis showed 7.9% bitumen having a penetration of 29.

Note in this example (as in Examples E and F) when voids are reduced, it is necessary for correct design to obtain "special lean Uvalde rock asphalt" in order that the total bitumen in the mixture may not be too high. Here with 18.0% voids (V) the total bitumen required was computed to be  $T=7.7\%$ . P. is said to be 5.5 to 6%—with a 5.5% bituminous rock the flux required was, of course, 2.2%. Look at the strength obtained—145 pounds shear. Actual analysis showed 7.9% bitumen in the mix which is in close agreement with the design.

This example shows correct design for low voidage, for percent total bitumen, and for selection of flux for controlling penetration. It should be contrasted with Example E, in which the flux was not properly selected.

The above tabulations will clearly illustrate the broad scope of the present invention. For specific illustration, Example F utilizes a rock asphalt containing approxi-

mately only 6% bitumen, which as before 65 pointed out, had never been employed to advantage as a base for paving material, for supposed lack of bitumen content. Rock asphalt with this lean content of bitumen, develops as indicated, excellent shear value 70 when fluxed with the proper penetration material.

By first determining the voidage of the crushed rock asphalt and the amount and penetration of the bitumen therein, the 75 amount and penetration of the flux to be added thereto may be definitely ascertained, the amount being based on that necessary to fill the voids, and the penetration being based on the final penetration desired relative to the amount added. It is necessary to determine the amount of bitumen contained in the crushed rock asphalt because the volume of the voids is to be filled by the volume of the bitumen contained in the rock asphalt 80 plus the volume of the added flux, and we cannot know the amount of flux required unless we know both the voids and the amount of bitumen in the rock asphalt. The penetration may readily be held where it 85 should be for best results in actual practice, and the amount of flux required is consistent with present fluxing ratios.

It may be pointed out that high stability and shear can be obtained by mixing the so-called lean (containing 5 to 6% bitumen) and the regular run rock asphalt (containing between 8 and 10% bitumen).

The penetration of the bitumen in the final mixture is an important item so far 100 as mixture stability is concerned, regardless of the kind of flux employed.

A comparison between Example A and Example F will indicate that by regulation of the crushing, the percentage of voids in 105 the rock asphalt after crushing, has been reduced from 23.2 to 18.6. This decrease in the voidage may be also brought about instead of, or in addition to, controlling the crushing operation as indicated in Example 110 G, in which the voids in aggregate have been reduced to 18.0% by adding a definite amount of desirable sized particles, which grading may not be obtained solely by crushing.

It may be pointed out that the percentage of bitumen in the final mixture is materially less in the mixture utilizing a relatively lean rock asphalt as compared with the mixtures using the relatively rich rock asphalts. The 120 resulting economy in the use of lesser quantities of flux to be added will be immediately apparent. This is obvious because in the light of the foregoing context it is seen that when the voids are reduced less bitumen is 125 required to fill them. With any grade of rock asphalt with a given percent bitumen, lowering the voids means simply that less

flux is added to the contained bitumen to fill the voids. With low void mixtures only lean rocks can be used, otherwise the voids are overfilled.

5 Since it is known that the most desirable stability values are inherent in such mixtures as have just sufficient bitumen to fill the voids, (the bitumen in the mixture is, of course, the naturally contained bitumen in 10 the rock asphalt plus the bitumen flux), and since the voids have been reduced in the mixtures described, it is apparent that the saving in flux is equal to the volume reduction in voids. Reducing the voids in any rock 15 asphalt simply means that the total bitumen required is less. In any rock asphalt of a given bituminous content the flux required to be added to the naturally contained bitumen is less when voids are reduced. Again, 20 if the voids are just filled with the total bitumen, it is obvious that the part added in the form of flux is, in itself, insufficient to fill the voids, but in the mixtures designed as 25 described in the examples cited, the bituminous flux added will, when added to the bitumen already contained in the rock asphalt, just fill said voids without substantial excess or deficiency.

It is strikingly shown that when mixtures 30 are properly designed on a voidage basis, a total bitumen content of .5 of 1% more than the theoretically correct amount of material reduces the shear strength materially.

It has been found that mixtures are most 35 stable when they contain the theoretically correct amount of bitumen. This sharp decline in resulting stability produces, of course, an inferior paving mixture.

Mixture stability is definitely controlled 40 by virtue of the grading of the crushed rock asphalt. The lower the voids, the greater the stability, provided the penetration of the bitumen is constant.

It is obvious from each of the examples 45 given that the difference between the computed bitumen content required to fill the voids in the aggregate and the self-contained bitumen in the rock asphalt is the amount of flux necessary to be added. The specification 50 states that the voids are found in order to compute the total bitumen required to fill them. These examples state the amount of bitumen already in the rock and the difference 55 is to be made up of flux, of course.

The preparation of a mixture in accordance 60 with the specifications outlined above may be carried out in any standard paving plant under approved methods as will be obvious. The flux may be added in heated condition and the crushed rock asphalt may or may not be heated prior to the introduction of the flux, or, as is obvious, the mixture may be prepared cold by utilizing a volatile solvent

for liquefying the added bituminous flux and the bitumen in the crushed rock asphalt. 65

I claim as my invention:

1. A method which comprises first determining the voidage in rock asphalt reduced to usable sizes, then adding bituminous flux in an amount insufficient to fill said voids 70 but in an amount which, when added to the naturally contained bitumen, is sufficient, with said naturally contained bitumen, to fill said voids without a substantial excess or substantial deficiency. 75

2. A method which comprises determining the voidage in rock asphalt, then reducing said voidage by grading, if necessary, to a minimum practicable for usability, then adding bituminous flux in an amount insufficient to fill said voids but in an amount which, when added to the naturally contained bitumen, is sufficient, with said naturally contained bitumen, to substantially fill 80 said voids without a substantial excess or substantial deficiency. 85

3. A method which comprises first determining the voidage in rock asphalt reduced to usable sizes, then adding bituminous flux in an amount insufficient to fill said voids 90 but in an amount which, when added to the naturally contained bitumen, is sufficient, with said naturally contained bitumen, to fill said voids without a substantial excess, or substantial deficiency, and controlling, by 95 selection, the consistency of said added flux to produce a mixture of a predetermined stability in which the total bitumen content has a predetermined penetration.

4. A method which comprises first determining the voidage in rock asphalt reduced to usable sizes, then adding bituminous flux in an amount insufficient to fill said voids but in an amount which, when added to the naturally contained bitumen, is sufficient, with said naturally contained bitumen, to fill 100 said voids without a substantial excess or substantial deficiency, liquefying the bitumen in said mixture and compacting the mixture in place to produce a bituminous 105 structure possessing high stability. 110

5. A method of preparing a bituminous composition which comprises reducing rock asphalt to usable sizes and determining the voidage thereof, then reducing said voidage by grading, if necessary, to a minimum practicable for usability by adding thereto bitumen-free or bitumen-impregnated mineral matter of desired sizes, and then adding a bituminous flux thereto in an amount insufficient to fill said voids but sufficient, when added to the bitumen naturally contained in the rock, to fill said voids without substantial excess or substantial deficiency. 115 120

In testimony whereof I affix my signature.  
WILLIAM P. BENTLEY.